

Patented July 6, 1926.

1,591,598

## UNITED STATES PATENT OFFICE.

HARRY M. WILLIAMS AND ALFRED L. BOEGEHOOLD, OF DAYTON, OHIO, ASSIGNEES TO  
GENERAL MOTORS RESEARCH CORPORATION, OF DAYTON, OHIO, A CORPORATION  
OF DELAWARE.

### PROCESS OF PRODUCING MALLEABLE IRON.

No Drawing.

Application filed May 21, 1924. Serial No. 714,892.

The present invention relates to improvements in making malleable iron castings and has among its objects, greatly cheapening the process and at the same time producing an excellent commercial malleable material.

Another object is to reduce to a small portion thereof, the time heretofore considered necessary to produce such castings.

The structural composition of malleable iron produced by the regular long anneal is a ferrite matrix containing nodules of temper carbon. The size of the ferrite grain, the number and size of the temper carbon nodules and their location relative to the ferrite grain, undoubtedly have a definite effect on the physical properties of the malleable iron. A certain amount of variation of these relations is permitted within the physical specifications for malleable iron. Properly annealed malleable iron contains no carbon in the combined form or in solution. There are but two metallographic constituents, namely ferrite and temper carbon.

The occurrence of the metallographic constituents in the form just described is a result of the composition and heat treatment of the iron. The first requirement of a casting intended for malleableizing is that it shall be of such composition that no free carbon will be precipitated in flake form during the solidification and subsequent cooling after casting. In other words, the casting must be white iron. The microstructure of such an iron is composed of primary dendritic crystals of austenite, and a secondary structure of austenite and massive cementite (iron carbide or  $Fe_3C$ ) in eutectic form. Upon annealing such a structure, the carbon is precipitated in the nodular form required for malleable iron. In the annealing of ordinary malleable iron, the first stage at  $1700^{\circ} F.$  changes the secondary structure in eutectic form of massive cementite and austenite into temper carbon in a matrix of austenite. After the massive cementite of the secondary eutectic structure has completely disappeared, further annealing at  $1700^{\circ} F.$  produces no change since approximately 1.3% carbon is soluble in iron at this temperature. The annealing temperature is then dropped very slowly to just below the lower critical temperature during which time the carbon in excess of eutectoid composition is progressively thrown out of solution in the

form of cementite, which is then decomposed into graphite and ferrite. The iron is then held at just below the lower critical temperature (approximately  $1340^{\circ} F.$ ) long enough for the eutectoid carbon, in form of cementite, to be precipitated and decomposed into ferrite and graphite in the form of temper carbon.

Silicon is the agent ordinarily used for causing the cementite to break down into iron and carbon. If the silicon content is too low, the time of annealing will be increased too much to make annealing commercially practicable. If the silicon is raised too high (above 1.3%) in the heretofore usual process in order to accelerate the annealing operation, there is danger of carbon precipitating in the form of flake graphite during the solidification of the casting. Even though this occurs to a very small extent, these flakes of graphite act as loci of carbon precipitation in the subsequent anneal, increasing the size of these flakes and consequently destroying the malleability of the casting. Therefore, commercially sand cast malleable iron must be held to a range of silicon content which requires long annealing periods to produce temper carbon.

Heretofore in producing malleable castings it has been the usual, if not the universal, practice to cast an article in an ordinary green sand mold, using an iron low in silicon in order to prevent the precipitation of carbon in flake form, and then put the cast article through an annealing cycle of about 110 hours, which cycle consists of (first) a heating up period of about 30 hours—during which time the articles are brought to a temperature of  $1700^{\circ} F.$ —(second) a period of about 40 hours—during which the temperature of  $1700^{\circ} F.$  must be maintained,— (third) slowly cooling to the lower critical temperature and holding this for about 35 hours, and (fourth) the period of cooling to a temperature low enough to permit handling, about five hours.

The present process, on the other hand, reduces the actual annealing time exclusive of heating and cooling from 75 hours, as required in the original process described to under 15 hours. Good results are obtained in four hours and can in some cases be reduced to two hours.

Contrary to the usual practice, it has been

- found that, if the carbon precipitating agent, such as silicon, is increased to from 2 to 4½%, the carbon maintained within the range of 1.7 to 3.5%, and the casting operation carried out in such a fashion as to obtain a white iron, the casting may then be converted to the malleable condition by annealing only a short time at a temperature of 1500 to 1700° F.
- 10 It has also been found that the content of the carbon precipitating agent, for example, silicon, bears a direct relation to the time required for annealing, the other conditions being maintained.
- 15 In carrying out the process which is based upon the foregoing discoveries, use is made of a mold in which the cooling of the casting may be controlled so as to accomplish this cooling very rapidly and thus obtain a product which is entirely white iron or one which is completely chilled. Solidification and cooling of the iron in the casting operation, through the temperature range where carbon is precipitated in flake form, or as flake graphite, should be as rapid as possible.
- 20 After the lower limit of this temperature range has been reached, the casting may be taken immediately to the annealing furnace or it may be allowed to cool to room temperature and subsequently annealed.
- 25 The preferred iron composition for reducing the annealing time to periods of 15 hours or less, will contain from 2 to 4½% silicon, 1.7 to 3.5% carbon, and a manganese, sulphur, and phosphorus content as low as practicable. The sulphur will be preferably not over .10 and phosphorus preferably not over .20%. The manganese content is preferably not over .70% but amounts
- 30 up to 1.00% do not seem to interfere greatly with the process.

If the silicon content is as low as 2%, the annealing time will be increased considerably but still be well below the time found necessary in the conventional or heretofore usual process.

A preferred iron composition is one that will require an annealing period of around four hours, and such a composition will have the silicon within the range of 2.5% to 3.25%, the carbon between 2.25% and 2.5% with the hereinbefore mentioned limits on manganese, phosphorus and sulphur.

The following specific compositions have been used and, when annealed for the time indicated, have given excellent quality malleable iron.

*Example No. 1.*

Carbon 1.76%, silicon 3.97%, sulphur .024%, phosphorus .004%, manganese .23%, iron the remainder. Annealing time—two hours.

*Example No. 2.*

Carbon 2.66%, silicon 2.77%, sulphur .031%, phosphorus .006%, manganese .18%,

iron the remainder. Annealing time—four hours.

As stated above the quantity of the carbon precipitating agent in the iron bears a direct relation to the length of the annealing time—as this quantity decreases the annealing time increases.

The quantity of carbon precipitating agent also bears a direct relation to the rate of cooling necessary to prevent graphite precipitation in flake form—as this quantity increases, the rate of cooling necessary to produce white iron, also increases, that is, the period of cooling becomes briefer.

From these two relations it is obvious that the best proportion of the precipitating agent will depend to some extent at least upon the efficiency of the mold in cooling the casting. If the mold is so designed that a given rate of cooling cannot be exceeded the proportion of the precipitating agent should be determined accordingly and it is from such relations that the preferred quantity mentioned hereinbefore has been determined, although it is obvious that a change in cooling rate occasioned by mold design will fix other proportions as the best in a given instance.

By controlling the solidification and subsequent cooling rate of the casting, it is possible to use much higher percentages of silicon than can be used in the process commonly practiced heretofore and at the same time not have carbon precipitation in flake form during the solidification and subsequent cooling. The microstructure of castings with the higher silicon percentages produced in the present process is identical with that of ordinary malleableizable iron casting before annealing. The extra silicon is present in solution in the iron and perhaps combined with the cementite and does not change the appearance of the constituents. When the casting is subsequently annealed, the high percentage of silicon causes the cementite to break down very rapidly into temper carbon and ferrite.

Among the carbon precipitating agents which may be used in the present process are silicon, aluminum, nickel, and copper, or combinations of these elements. Silicon may be considered as the preferred one and has been given in the specific examples.

Further, although it has been indicated above that, when casting the iron to be malleableized, conditions should be controlled so as to produce a white iron, it should be noted that any precipitation of carbon during the casting operation will not interfere with the annealing unless it precipitates in the flake graphite form. Precipitation of nodular carbon at this period is not objectionable.

Finally, it should be noted that the invention is not to be limited to the precise

proportions and procedure mentioned as these may undoubtedly be varied within the scope of the claims which follow.

What is claimed is as follows:

- 5 1. The process of making malleable iron castings which consists in pouring into a mold iron containing a carbon precipitating constituent; cooling the casting at such rapid rate as to prevent precipitation of flake graphite; and then annealing the casting; the proportion of carbon precipitating constituent being substantially in excess of that which can be included in malleableizable iron poured in sand molds and cooled at the usual rate.
- 10 2. The process of making malleable iron castings which consists in pouring into a chill mold, iron containing a proportion of carbon precipitating constituent substantially in excess of the amount that can be included in malleableizable iron poured into sand molds, and then annealing the casting.
- 15 3. The process of making malleable castings which consists in making a white iron casting from an iron mixture containing more than 1.3% silicon, then annealing the casting.
- 20 4. The process of making malleable iron castings which consists in preparing a molten mixture of iron containing more than 1.3% of silicon; pouring the molten mixture into a mold of sufficiently high heat conductivity to chill the casting so rapidly that substantially no flake carbon will be precipitated, then annealing the casting.
- 25 5. The process of making malleable iron castings which consists in pouring into a chill mold, molten iron containing from 2.00 to 4.50% silicon, then annealing the casting.
- 30 6. The process of making malleable iron castings which consists in pouring into a

metallic mold, molten iron containing more than 1.70% of carbon and more than 1.3% of silicon, then annealing the casting.

45

7. The process of making malleable iron castings which consists in pouring iron containing from 2% to 4.50% silicon and 1.70% to 3.50% carbon into a metallic mold and subsequently annealing the casting.

50

8. The process of making malleable iron castings which consists in preparing a molten mixture of iron containing upward of 1.70% of carbon and upwards of 2% of silicon, pouring the molten mixture into a mold of sufficiently high heat conductivity to chill the casting so rapidly that substantially no flake carbon will be precipitated, then annealing the casting at a temperature of about 1500° to 1700° F. for a period not exceeding fifteen hours.

55

9. The process of producing malleable iron articles which consists in casting the article of iron containing from 2.00 to 4.50% Si, 1.70 to 3.50% C, and as low as practicable in Mn, P and S content under conditions to give a white iron and subsequently annealing for a short period of time.

60

10. The process of producing malleable iron articles which consists in casting the article in a metallic mold and subsequently annealing for a short period of time.

70

11. The process of producing malleable iron articles which consists in casting the article of iron containing from 2.00 to 4.50% Si, 1.70 to 3.50% C, and as low as practicable in Mn, P, and S content in a metallic mold and subsequently annealing for a short period of time.

75

In testimony whereof we hereto affix our signatures.

80

HARRY M. WILLIAMS.  
ALFRED L. BOEGEHOOLD.